

June 7, 1927.

1,631,623

A. W. COCHRAN

METHOD OF FORMING CUTTING TOOLS

Filed July 13, 1925



Inventor:  
Albert W. Cochran  
General & Ramsey  
By Atty.s

## UNITED STATES PATENT OFFICE.

ALBERT W. COCHRAN, OF PORTLAND, OREGON.

## METHOD OF FORMING CUTTING TOOLS.

Application filed July 13, 1925. Serial No. 43,285.

My invention relates to the forming of metal tools with cutting edges by drop forging or by other method, utilizing compression dies or members which serve to diminish, in cross section, the blank of material being formed. I have discovered that if a blank of material, and the dies or members, are so relatively arranged, that the cutting edge to be formed, is placed at the parting line between said dies or members, through which the excess material is forced by the compression, the grain structure in the cutting edge will be elongated transversely, to produce an extremely tough and strong edge. That is, I have discovered that I can produce a tool with a tough edge, such as is produced by hand-hammering a cutting edge merely by arranging the die halves so that the parting line forms a continuation of the portion of the recess therein which produces the cutting edge. The arranging of the recesses in the die halves in this manner tends to produce a flow of the excess material expressed from between said die halves through the portion of the die which forms said cutting edge.

The details of this method and of the die elements are hereinafter described in greater detail, reference being made to the accompanying drawings, in which:

Fig. 1 is a diagrammatic section through two die halves, spaced apart, and with a blank of material arranged therein;

Fig. 2 is a similar section showing the die halves as having been compressed, to form the tool and to express the excess material; and

Fig. 3 is a plan view of the material after being so compressed showing how the tool is blanked in, and a relatively thin fin of material is formed thereabout, by the excess material.

My invention is particularly adapted to drop-forging operations and the dies used therein, although it is also adapted to be used in press work and other dies, or members, which use compression solely, such, for example, as forming dies and forming rolls. Where I refer to compression dies and compression members, I thus wish to include not only dies used for drop-forging but also forming dies and forming rolls which do not utilize impact, in addition to compression.

As shown in Fig. 1, the two die halves *a* and *b* are formed to have companion recesses *c* and *d*, which are each substantially one-

half of the shape of the tool to be formed. The parting lines between the recesses, so formed, constitute virtually a continuation of said recess and preferably does not diminish, substantially, in thickness. Thus, for example, in Fig. 2, the recess formed between said two die halves by the companion recesses *c* and *d* might be said to terminate at the lines *A*—*A* and *B*—*B* and the remainder of space outside of said lines constitute the parting lines *e* and *f*. Thus when a blank of material *g* is placed between the die halves, which are spaced apart, the compression of said die halves produces a fin of material *g'* about the body *g''* of the tool being formed, because a blank of material is used which is substantially larger than the ultimate tool to be formed. Thus the configured blank, as shown in Fig. 3, must be trimmed so as to remove the entire fin *g'* therefrom. This is done, however, with the ordinary die used to remove a fin from any drop forging. A tool made in this manner must be dressed to remove the scale and also to sharpen the edge. The tool, however, is made so as to be substantially the same size as the ultimate dressed tool, sufficient material being provided merely to permit the scale, caused by the heating of said blank, to be removed and the cutting edge to be sharpened. By producing a tool in this manner a cutting edge is provided which has been formed or forged as compared with one which has been milled or ground.

The tool which I show in the drawings is used as a router bit in cutting away the excess material from stereotype plates and the like, and is the subject of a co-pending application. Tools of this character require a very tough edge because they are driven at a tremendously high rate of speed which wears an edge away very quickly and also tends to break off portions if forced into the work too quickly. Tools similar to these are sold on the market at present, but said tools are ground or milled to size from a blank. By operating one of said tools alongside of a tool made by my improved method, I have discovered that the ground or milled tool will not hold an edge more than half as long as one made by my method.

I am aware that it is old to produce a cutting edge such as a razor edge by hand forging, that is, by drawing said edge out with a hammer and thus do not wish to claim this manner of producing a cutting

edge. My invention is limited entirely to die elements for forming and to the producing of a cutting edge between two compression members, such for example, as the halves of a die used in drop forging or the halves of a forming die, or forming rolls.

It is to be particularly noted that the die members confine the outflow of the excess metal to a point coincident with and extending materially beyond the parting line so as to insure that the grain of the metal will be elongated transversely of the cutting edge without possibility of that distortion in the grain which would probably follow the interruption of the confining area of the dies exactly at the parting line. In the latter instance, the unconfined flow of the excess metal substantially at the parting edge would tend to a distortion of the grain formation and certainly could not result in the even distribution and elongation of the grain directly transverse what is to be the cutting edge of the tool in final form. By continuing the confinement of the metal beyond this parting or subsequent cutting edge of the tool, there is no liability of grain distortion at such edge.

I claim:

1. The improved method of producing a

cutting tool consisting in placing a block of metal between companion dies whose working faces are shaped to form the tool to and including the cutting edge thereof and extended beyond said cutting edge to confine the flow of excess metal in substantial uniformity with the confinement at the cutting edge, whereby the grain of the metal is elongated through and beyond the cutting edge line to insure that said grain structure will be elongated transversely at the cutting edge line.

2. The improved method of producing a cutting tool with a curved edge consisting in placing a block of metal of greater cross section than that to be given the tool between companion dies whose working faces are curved and spaced from each other in conformity with the cross section and the curve to be given the tool in the direction of its edge and said dies being adapted to confine the outflow of the excess metal to an opening coinciding with the parting line at the cutting edge of the tool, whereby the grain of the metal in the curved section of the tool is approximately uniformly elongated in the direction of its taper and towards its edge.

ALBERT W. COCHRAN.